

April 30, 1946.

W. G. ABBOTT, JR.

2,399,191

## PRODUCTION OF SLIVERS OF ARTIFICIAL FIBERS

Filed Oct. 18, 1943



Fig. 3

Trevenor  
William G. Abbott Jr.  
By Polk, Cushman & Good  
att'ys.

## UNITED STATES PATENT OFFICE

2,399,191

## PRODUCTION OF SLIVERS OF ARTIFICIAL FIBERS

William G. Abbott, Jr., Milford, N. H.

Application October 18, 1943, Serial No. 506,684

5 Claims. (CL 18—54)

This invention relates to the production of slivers consisting of artificial fibers of staple length staggered and overlapped in the sliver, such, for example, as would be suitable for spinning either directly or after drawing.

The practical method of forming artificial fibrous material by extrusion is to extrude the material in liquid or plastic form through a spinneret having a considerable number of minute orifices and harden the material by one of several operations such as causing coagulation of the material in a bath, or permitting a solvent for the material to vaporize, or permitting a material of a thermoplastic nature to cool.

The sliver so produced can be cut into staple lengths and worked on to distribute the pieces of fibers lengthwise in proper overlapping relation. It has been proposed to avoid the cutting operation by intermittently interrupting the flow of liquid material to the orifices of a spinneret so as to produce initially a discontinuous sliver consisting of sections each of staple length. But with such a proposed procedure the sliver after its formation would still need to be mechanically treated to distribute the fibers thereof in proper overlapping relation lengthwise of the sliver.

The present invention aims to avoid the necessity for distributing the staple lengths of fibers after the formation of the sliver, and aims to form the sliver, in the first instance, with its individual fibers of staple length and properly overlapped and distributed lengthwise in the sliver.

Other objects and advantages of the invention will be apparent from the specification and its drawing, wherein the invention is described and illustrated by way of example.

In the drawing

Fig. 1 is a schematic view of a preferred form of apparatus for practicing the invention;

Fig. 2 is a vertical sectional view, enlarged but not to scale, through a spinneret and coagulating bath, diagrammatically showing the fibers being formed from a composite in which the filament-forming material constitutes the dispersed phase; and

Fig. 3 is a view similar to Fig. 2 showing the fibers being formed from a composite in which the filament-forming material constitutes the continuous phase.

Referring to the drawing, a spinneret 11 is provided, and may be of conventional form, containing the desired large number of extrusion orifices of such number and size as will produce the desired sliver.

5 A suitable coagulating solution 12 is maintained in a tank 13 into which the spinneret 11 discharges the extruded material, the coagulating solution being of such nature as to solidify the fiber-forming substance of the extruded material.

As applied to the extrusion of a solution of viscose, the coagulating bath may, for example, consist of:

|                       | Per cent |
|-----------------------|----------|
| Acid                  | 9        |
| Sodium sulphate       | 15       |
| Zinc sulphate         | 1        |
| Corn sugar or glucose | 6        |

15 in aqueous solution.

The spinneret 11 may be supplied with material by suitable means such as a pump 14 receiving its supply from a tank 15. The tank 15 is preferably provided with agitating mechanism, such, for instance, as a motor-driven propeller 16, adapted to maintain the material in a thoroughly mixed condition, as more fully explained below.

20 According to the invention, the material of which the filaments are to be formed, for example viscose, is maintained in the supply tank 15 in a composite which includes another material which retains its separate identity in the mixture and is separable from the filament-forming material after extrusion. Where, as in this example of the invention, the filament-forming material is hardened by coagulation, the separation of the other material from the filament-forming material after extrusion is most easily accomplished by employing as the other material a material which is not subject to be coagulated by the coagulating bath and which will either settle to the bottom or rise to the surface of such bath.

25 The viscose may, for example, constitute the dispersed phase of the composite. As the continuous phase of the composite, suitable for use with viscose, there may be employed a light mineral oil or naphtha which will separate from the coagulating bath by rising to the surface, or a liquid such as carbon disulphide that will separate from the coagulating bath by collecting at the bottom of the tank 13.

30 As the material from the supply tank is forced through the extrusion orifices of the spinneret, the particles of viscose solution passing through each orifice are separated lengthwise by the other, removable and non-coagulable, ingredient 35 of the composite. Upon entry into the coagulat-

ing bath, the separate particles of filament-forming viscose material are then coagulated into separate fibers of staple length.

Fig. 2 shows in a diagrammatic way liquid filament-forming coagulable particles 20 of viscose, constituting the dispersed phase of the composite approaching and passing through some of the extrusion orifices, and then being acted on as separate filaments 20<sup>a</sup> by the coagulating solution 12. Fig. 2 also shows the flow of filament-forming particles interrupted at the moment at some of the orifices by the passage through those orifices of non-coagulable liquid 21 constituting the continuous phase of the composite. This figure also indicates diagrammatically how the separate filaments 20<sup>a</sup> of the sliver are overlapped and staggered longitudinally of the sliver. It will be understood that this figure shows only a few of the many streams of composite which are extruded simultaneously.

Fig. 3 shows in a diagrammatic way the use of a mixture in which the filament-forming coagulable viscose, indicated at 20, constitutes the continuous phase, with the other material 21, separable from the filament-forming material after extrusion, constituting the dispersed phase, and the formation of the separate filaments 20<sup>a</sup> in a manner similar to Fig. 2.

Whether the filament-forming material constitutes a dispersed phase, as in Fig. 2, or a continuous phase, as in Fig. 3, the filament-forming material and the other material are so disposed, substantially uniformly throughout the composite, the bodies of each material will be presented to the individual orifices at frequent intervals, the bodies of said other material filling the orifice cross-section to the temporary exclusion of the filament-forming material.

Because of the considerable number of extrusion orifices in the spinneret and the intimate mixture between the filament-forming material and the other material, the resulting staple length fibers are distributed fairly evenly lengthwise of the sliver. The sliver so produced consists of a number of parallel laid fibers, of staple but more or less uneven length, overlaid in a more or less uneven pattern, the sliver itself being of fairly uniform weight and diameter along its length.

Preferably, in order to insure even action of the coagulating solution on the material and to hold the fibers together loosely while they are being hardened by coagulation and the other material of the composite is being separated from them, they are confined laterally in the coagulating bath by a tube 25, which may be perforated. A suitable amount of twist can be imparted to the sliver by a relative rotation of the spinneret 11 and tank 13 in which the sliver is formed. For simplicity, the tank 13 is shown as mounted for rotation with a turntable 27. Such rotation of the coagulating tank 13 not only serves to impart the desired slight twist to the sliver, but also serves to coil the sliver in a fairly even form at the bottom of the tank.

The invention is also applicable to processes in which no twist is imparted to the sliver, and various forms of means may be employed to hold the sliver together during hardening and subsequent washing.

During the coagulating action, the coagulating solution may be replenished or changed by the addition of further coagulating solution through an entrance pipe 30, and excess solution may be allowed to discharge either continuously or inter-

mittently through an overflow pipe 31 leading from the bottom of the tank. A perforate diaphragm 32, slightly above the entrance of the overflow pipe 31, serves to support the coils of formed sliver and prevent these from obstructing the entrance to the overflow pipe. A circular trough 33 surrounding the upper end of the rotatable tank 13 is provided to catch the overflow from pipe 31.

Although for simplicity of illustration the apparatus is shown as being of the type that requires periodic removal of the sliver from tank 13, the invention is similarly applicable to processes in which the sliver is delivered from the apparatus continuously.

The form of the resulting sliver can be varied by suitable control of the volume of filament-forming material supplied to the spinneret, the relative proportions of the filament-forming material and the other material of the composite, the relative sizes of the particles of these materials as they pass through the extrusion orifices, and the number and size of extrusion orifices, so as to produce slivers of the nature of top slivers and roving slivers of various sizes and weights.

Moreover, instead of a single filament-forming substance, two or more distinct filament-forming substances may be included in the composite, so as to form a sliver in which fibers of different chemical and mechanical structure are blended together.

For example, the composite may have two dispersed phases. One of such dispersed phases may be, for example, casein suitably prepared and reduced to a viscous syrup by an aqueous solution of sodium hydroxide. A second dispersed phase may consist of zein, which is a corn product protein which after purification is dissolved in alcohol or carbitol to form a thick syrup. These two dispersed phases are preferably dispersed separately in the continuous phase non-coagulable material which may consist of a light coal tar naphtha or heavier chlorinated product in which these dispersed phases are insoluble, and the whole composite thoroughly mixed. As a coagulating bath for forming this blended sliver, a solution of formaldehyde and water may be employed, and to such solution there may be added acetic acid, glucose or calcium chloride in order to assist the coagulation and hardening of the filaments.

While the mixture has been described by way of example as utilizing a liquid as the other material, separable from the filament-forming material after extrusion, the mixture may utilize gases or semi-solid material for the same purpose.

To further illustrate the invention, it may be applied to filament-forming material that is hardened after extrusion by vaporization of a volatile solvent rather than by use of a coagulating bath. Thus cellulose acetate dissolved in acetone may constitute the filament-forming material, the acetone may be allowed to vaporize to solidify the cellulose acetate, and the other material of the mixture, which retains its separate identity in the composite, may consist of a waxy hydrocarbon of liquid consistency and be removed from the sliver by treatment by a solvent.

The invention may also be applied to thermoplastic filament-forming material that is extruded in a plastic condition. Thus, nylon or Vynylon may constitute the filament-forming material and may solidify by cooling after the extrusion of the mixture, and the other material of the mixture may be removed from the sliver by treat-

ment by a solvent. In the extrusion of composites in which the filament-forming material is in a plastic condition, it is preferred that the other material of the composite be of a plastic nature, such, for example, as a plastic waxy hydrocarbon. As in the other forms of the invention, the materials of the composite are selected so as to retain their separate identities in the mixture.

I claim:

1. Method of forming a sliver of artificial fiber which comprises forming a composite of filament-forming material and another material, both said materials being in a flowable condition and being immiscible with each other so that each retains its separate identity, continuously feeding said composite through a plurality of adjacent orifices adapted to extrude the plurality of filaments which together constitute a sliver, said materials being so disposed, substantially uniformly throughout the composite, as to present bodies of each material to the individual orifices at frequent intervals, the bodies of said other material filling the orifice cross section to the temporary exclusion of the filament-forming material, whereby to produce a sliver from the several orifices comprising pieces of filament-forming material overlapped and staggered longitudinally of the sliver, and after passage through the orifices separating said other material from the filament-forming material.

2. Method of forming a sliver of artificial fiber which comprises forming a composite of filament-forming material and another material, both said materials being in a flowable condition and being immiscible with each other so that each retains its separate identity, continuously feeding said composite through a plurality of adjacent orifices adapted to extrude the plurality of filaments which together constitute a sliver, said materials being so disposed, substantially uniformly throughout the composite, as to present bodies of each material to the individual orifices at frequent intervals, the bodies of said other material filling the orifice cross section to the temporary exclusion of the filament-forming material, whereby to produce a sliver from the several orifices comprising pieces of filament-forming material overlapped and staggered longitudinally of the sliver, and after passage through the orifices separating said other material from the filament-forming material while confining the sliver laterally.

3. Method of forming a sliver of artificial fiber which comprises forming a composite of filament-forming material and another material, both said materials being in a flowable condition and being immiscible with each other so that each retains its separate identity, continuously feeding said composite through a plurality of adjacent orifices adapted to extrude the plurality of filaments which together constitute a sliver, said materials

being so disposed, substantially uniformly throughout the composite, as to present bodies of each material to the individual orifices at frequent intervals, the bodies of said other material filling the orifice cross section to the temporary exclusion of the filament-forming material, whereby to produce a sliver from the several orifices comprising pieces of filament-forming material overlapped and staggered longitudinally of the sliver, and after passage through the orifices separating said other material from the filament-forming material and applying a twist to the sliver.

4. Method of forming a sliver of artificial fiber which comprises forming a composite of a plurality of filament-forming materials and another material, all of said materials being in a flowable condition and the said other material being immiscible with the filament-forming materials so that said other material retains its separate identity, continuously feeding said composite through a plurality of adjacent orifices adapted to extrude the plurality of filaments which together constitute a sliver, said materials being so disposed, substantially uniformly throughout the composite, as to present bodies of the filament-forming materials and bodies of said other material to the individual orifices at frequent intervals, the bodies of said other material filling the orifice cross section to the temporary exclusion of the filament-forming material, whereby to produce a sliver from the several orifices comprising pieces of filament-forming material overlapped and staggered longitudinally of the sliver, and after passage through the orifices separating said other material from the filament-forming material.

5. Method of forming a sliver of artificial fiber which comprises forming a composite of a plurality of filament-forming materials in dispersed phase and another material in continuous phase, all of said materials being in a flowable condition and the said other material being immiscible with the filament-forming materials so that said other material retains its separate identity, continuously feeding said composite through a plurality of adjacent orifices adapted to extrude the plurality of filaments which together constitute a sliver, said materials being so disposed, substantially uniformly throughout the composite, as to present bodies of the filament-forming materials and bodies of said other material to the individual orifices at frequent intervals, the bodies of said other material filling the orifice cross section to the temporary exclusion of the filament-forming material, whereby to produce a sliver from the several orifices comprising pieces of filament-forming material overlapped and staggered longitudinally of the sliver, and after passage through the orifices separating said other material from the filament-forming material.

WILLIAM G. ABBOTT, JR.